

Jan. 5, 1932.

J. J. FINGLAND ET AL

1,840,028

## PROCESS FOR REFINING LEAD BISMUTH ALLOYS

Filed May 9, 1929



FIRE  
L

John J. Flanagan  
Alexander D. Turnbull  
Peter F. McIntyre  
for Chas. A. Nichols  
Attorney

## UNITED STATES PATENT OFFICE

JOHN JAMES FINGLAND, ALEXANDER DOUGLAS TURNBULL, AND PETER FINDLAY MCINTYRE, OF TRAIL, BRITISH COLUMBIA, CANADA, ASSIGNORS TO THE CONSOLIDATED MINING AND SMELTING COMPANY OF CANADA, LIMITED, OF MONTREAL, QUEBEC, CANADA, A COMPANY OF CANADA

## PROCESS FOR REFINING LEAD-BISMUTH ALLOYS

Application filed May 9, 1929. Serial No. 361,834.

Our invention relates to a process of refining lead-bismuth alloy, containing 20-40% bismuth, which comprises heating a charge of the crude alloy to a temperature above its 5 fusing point, adding zinc to the molten charge, agitating it at that temperature, slowly cooling it, by successive stages, progressively graduated from the maximum temperature of the charge to the freezing 10 point of the residual lead-bismuth alloy, and removing at each stage, the solidifying metals and impurities, for the production at the final stage of a low freezing lead-bismuth alloy, substantially free from the other metals 15 and impurities with which it was associated at the initial stage of the operation.

The refining of the alloy may be conducted by effecting the heating and the subsequent 20 succession of coolings in a single receptacle but it is more practical to conduct them separately in a plurality of heated receptacles arranged in differential thermal-series definitely graduated between the maximum and 25 minimum temperatures of the operation, and transfer the solidifying metals and impurities, in the form of crusts, from the cooler to the hotter receptacles and the liquid metal from the hotter to the cooler receptacles, until a residual liquid lead-bismuth 30 alloy is obtained in the last receptacle of the series free or substantially free from other metals and impurities, including the zinc, added to the charge at the initial stage of the 35 operation.

A suitable plant for carrying out the process, shown diagrammatically in the accompanying drawing, may consist of a battery 40 of six 5-ton kettles, at one end of which is a firebox for providing the necessary heat with provision for conducting the gaseous products of combustion around each kettle in succession and thence to the stack; the heating arrangements being sufficient to maintain 45 1100° F. in the first kettle and 400° F. in the last kettle of the series, and the actual procedure being carried out as follows:—

A charge of crude lead-bismuth alloy is heated to a temperature of about 1000° F. 50 in the second kettle and from 1½ to 3% zinc is added to the molten charge which is

agitated with a mechanical stirrer at that temperature. The successive crusts of the second kettle are transferred to and accumulated in the first kettle until it contains a full charge from a number of like operations. 55 The charge in the first kettle, is re-melted and stirred at a temperature of about 1100° F. and the crusts are removed from it and separately treated by known metallurgical methods for the recovery of their valuable contents, including the added zinc. The residual liquid metal from the first kettle is returned to the second kettle as part of a succeeding charge and the liquid metal in the second kettle, when the crust has been removed from it, is transferred to the third kettle heated to a temperature ranging between 800° and 900° F. As cooling proceeds the crust is transferred from the third kettle to the second kettle for retreatment 70 with a subsequent charge in the second kettle, and the liquid metal in the third kettle is transferred to the fourth kettle heated to a temperature ranging from 600° to 700° F. The crust of the fourth kettle is transferred 75 to the third kettle and the liquid metal in the fourth kettle is transferred to the fifth kettle heated to a temperature ranging between 300° and 500° F. The crust of the fifth kettle is transferred to the fourth kettle 80 and the liquid metal in the fifth kettle is transferred to the sixth kettle to give a low freezing liquid lead-bismuth alloy free or substantially free from other metals and impurities.

The application of this procedure 85 finally resolves the original charge into two products; one of which consists of lead-bismuth alloy, free or substantially free from impurities and from other metals such as gold, silver, arsenic, antimony, and added zinc, suitable for the recovery of bismuth by electrolytic or other metallurgical operations; and another which consists chiefly of the other metals contained in the crude charge such as gold, silver, arsenic and antimony together with the added zinc and small proportions of lead and bismuth, to be treated by known metallurgical methods 95 for the recovery of the valuable contents.

The following example indicates the com- 100

position of the crusts and liquid metals, and the analytical results secured from representative samples taken at a period when the system of separation was in complete action during the treatment of 88 tons of the crude material containing 109.4 ozs. gold, 16684 ozs. silver, 59% lead, 28% bismuth, a trace of arsenic, and 0.25% antimony, together with the addition of 2½% zinc.

|                            | Gold—<br>ozs. per<br>ton | Sil-<br>ver—<br>ozs. per<br>ton | Zinc % | Temp.<br>°F. |
|----------------------------|--------------------------|---------------------------------|--------|--------------|
| 10                         |                          |                                 |        |              |
| 15 Crusts kettle:          |                          |                                 |        |              |
| #2 passing to kettle #1    | 4.12                     | 1786.6                          | 20.0   | 1100-900     |
| #3 passing to kettle #2    | 0.54                     | 969.6                           | 16.0   | 900-800      |
| #4 passing to kettle #3    | 0.03                     | 617.4                           | 15.3   | 700-600      |
| #5 passing to kettle #4    | Trace.                   | 115.0                           | 8.6    | 500-300      |
| Liquids kettle:            |                          |                                 |        |              |
| #2 passing to kettle #3    | 0.03                     | 235.5                           | 6.0    | -----        |
| #3 passing to kettle #4    | 0.01                     | 93.6                            | 3.7    | -----        |
| #4 passing to kettle #5    | Trace.                   | 14.1                            | 1.5    | -----        |
| 20 #5 passing to kettle #6 | Trace.                   | Trace.                          | NH.    | -----        |

Having thus fully described our invention what we claim as new and desire to secure by Letters Patent is:

25 1. A process of refining lead-bismuth alloy containing 20-40% bismuth, which comprises incorporating zinc with a charge of the crude alloy in a fusing vessel, heating it, maintaining the heat at an uniform temperature throughout the charge materially above its fusion point, transferring the crust of the molten charge to a separate vessel uniformly heated to a higher temperature than said fusing vessel and the liquid residue of the charge to a succession of separate vessels, the temperatures of which are progressively graduated from the maximum of the graduated temperatures to the freezing point of the residual lead-bismuth alloy, maintaining each vessel at an uniform temperature throughout the charge, transferring the solidifying metals and impurities from each of the lower heated vessels to the next higher heated vessel in succession and transferring the liquid residue from each of the higher heated vessels to the next lower heated vessel in succession for the production, at the lowest heated vessel, of a low freezing lead-bismuth alloy substantially free from the other metals and impurities with which it was associated at the commencement of the operation.

40 2. A process of refining lead-bismuth alloy containing 20-40% bismuth, which comprises incorporating zinc with a charge of the crude alloy in a fusing vessel, heating it and maintaining the heat at a substantially uniform temperature of 1000° F. throughout the charge, transferring the crust of the molten charge to a separate vessel uniformly heated to a temperature of substantially 1100° F. and the liquid residue of the charge to a succession of separate vessels the temperatures of which are progressively graduated from 900° F. to 300° F., maintaining each

vessel at an uniform temperature throughout the charge, transferring the solidifying metals and impurities from each of the lower heated vessels to the next higher heated vessel in succession and transferring the liquid residue from each of the higher heated vessels to the next lower heated vessel in succession for the production, at the lowest heated vessel, of a low freezing lead-bismuth alloy substantially free from the other metals and impurities with which it was associated at the commencement of the operation.

45 3. A process of refining lead-bismuth alloy containing 20-40% bismuth, which comprises incorporating from one and one half per cent to three per cent of zinc with a charge of the crude alloy in a fusing vessel, heating it, maintaining the heat at an uniform temperature throughout the charge, transferring the solidifying metals and impurities from each of the lower heated vessels to the next higher heated vessel in succession and transferring the liquid residue from each of the higher heated vessels to a separate vessel uniformly heated to a higher temperature than said fusing vessel and the liquid residue of the charge to a succession of separate vessels, the temperatures of which are progressively graduated from the maximum of the graduated temperatures to the freezing point of the residual lead-bismuth alloy, maintaining each vessel at an uniform temperature throughout the charge, transferring the solidifying metals and impurities from each of the lower heated vessels to the next higher heated vessel in succession and transferring the liquid residue from each of the higher heated vessels to the next lower heated vessel in succession for the production, at the lowest heated vessel, of a low freezing lead-bismuth alloy substantially free from the other metals and impurities with which it was associated at the commencement of the operation.

50 4. A process of refining lead-bismuth alloy containing 20-40% bismuth, which comprises incorporating from one and one half per cent to three per cent of zinc with a charge of the crude alloy in a fusing vessel, heating it and maintaining the heat at a substantially uniform temperature of 1000° F. throughout the charge, transferring the crust of the molten charge to a separate vessel uniformly heated to a temperature of substantially 1100° F. and the liquid residue of the charge to a succession of separate vessels the temperatures of which are progressively graduated from 900° F. to 300° F., maintaining each vessel at an uniform temperature throughout the charge, transferring the solidifying metals and impurities from each of the lower heated vessels to the next higher heated vessel in succession and transferring the liquid residue from each of the higher heated vessels to the next lower heated vessel in succession for the production, at the lowest heated vessel, of a low freezing lead-bismuth alloy substantially free from the other

metals and impurities with which it was associated at the commencement of the operation.

5. A process of refining lead bismuth alloy containing 20-40% bismuth by passing the charge through a series of separate thermal stages; which comprises incorporating zinc in a charge of the crude alloy; heating the charge at the initial stage to a temperature ranging between 900° F. and 1100° F.; removing the solidifying metals and impurities from the molten charge at the initial stage and transferring them to the crust melting stage and there heating them to a higher temperature than that of the initial stage; removing the liquid residue from the initial stage and passing it through a succession of separate thermal stages of progressively descending temperatures graduated from 900° F. to 300° F.; maintaining an uniform temperature throughout the charge at each stage; removing the solidifying metals and impurities at each stage and transferring them to the next higher heated stage of the series for the recovery of all the contained metals except the lead and bismuth; and removing the liquid residue at each stage and transferring it to the next lower heated stage of the series for the production at the lowest thermal stage of a low freezing lead bismuth alloy substantially free from the other metals and impurities with which it was associated at the commencement of the operation.
- 35 6. A process of refining lead bismuth alloy containing 20-40% bismuth which comprises incorporating zinc in a charge of the crude alloy, passing the charge through a series of separate thermal stages of progressively descending temperatures graduated from 1100° F. to 300° F.; maintaining at each stage an uniform temperature throughout the charge, passing the solidifying metals and impurities from each stage to the next higher stage of the series and the residual liquid from each stage to the next lower stage of the series; and recovering, at the final stage at one end of the operation, a low freezing lead bismuth alloy substantially free from the other metals and impurities with which it was associated at the commencement of the operation, and at the final stage at the other end of the operation a crust containing said other metals and impurities.
- 55 Signed at the city of Trail, Province of British Columbia, this 31st day of March, A. D. 1929.

JOHN JAMES FINGLAND.

PETER FINDLAY McINTYRE.

ALEXANDER DOUGLAS TURNBULL.